

Dec. 15, 1964

W. H. KINGSLEY ET AL

3,161,540

PROCESS OF MANUFACTURING INSULATED HEATER WIRE AND ARTICLE

Filed June 20, 1962



Fig. 1



Fig. 2

INVENTORS  
Wayne H. Kingsley &  
Douglas S. Monroe  
BY  
Robert E. Strausser  
ATTORNEY

1

3,161,540

PROCESS OF MANUFACTURING INSULATED  
HEATER WIRE AND ARTICLE  
Wayne H. Kingsley and Douglas S. Monroe, Emporium,  
Pa., assignors to Sylvania Electric Products Inc., a cor-  
poration of Delaware  
Filed June 20, 1962, Ser. No. 203,962  
6 Claims. (Cl. 117—217)

This invention relates generally to the manufacture of an insulated wire and more particularly to a process for forming an insulated wire which may be used as a heater for an electron discharge device.

In the manufacture of heaters for electron discharge devices, the process of depositing a binder suspension containing aluminum oxide upon a refractory wire to provide a conductor having an insulating layer of aluminum oxide has been extensively used for a number of years. In this process, it has been found that refractory wires such as tungsten have a multitude of surface contaminants and oxides which must be removed before adequate adherence of the insulating layer can be obtained. Accordingly, the wire is heated in a reducing atmosphere prior to the addition of the insulating layer to substantially remove the surface contaminants and oxides.

Thereafter, a layer or multiple layers of the binder suspension containing the aluminum oxide are deposited on the cleaned wire. Further, during this period of suspension deposition or shortly thereafter, the coated wire is subjected to heat in order to remove the volatile constituents of the binder and cause the aluminum oxide to adhere to the refractory wire. During this coating process, it has been found that the heat necessary for the removal of the volatile binder constituents and to cause adherence of the aluminum oxide to the wire is within the range of the heat at which oxides are formed on the refractory wire. The deleterious presence of oxides on the wire during the manufacturing process is difficult to detect and control and their presence results in excessive wire loss and increased expense due to poor adherence of the insulating layer. Additionally, it is believed that oxides between the wire core and the insulating layer provide the basis for electrical leakage between the heater and the cathode of an electron tube, increased hum when the heater is activated by an A.C. voltage, and eventual "burn out" or failure of the heater during sustained operation.

Therefore, it is an object of this invention to improve the adherence between the refractory wire and a layer of insulation provided thereon.

Another object of this invention is to improve the permissible range of operating heat employed during the process of depositing a layer of insulating material on a refractory wire.

A further object of this invention is to reduce the leakage current level between the heater and the cathode in an indirectly heated electron discharge device.

A still further object of this invention is to enhance the life characteristics of an electron discharge device.

The foregoing objects are achieved in one aspect of this invention by the provision of a noble metal barrier film intermediate the refractory wire and the layer of insulating material to inhibit oxide formation on the wire as well as any chemical reaction between the binder constituents of the deposited layer and any oxides formed on the wire during the insulator forming operation.

It is to be understood that any refractory metal wire which may be used as a heater in an electron discharge device is applicable to this manufacturing operation although tungsten, molybdenum and alloys thereof are preferable. Further, the noble metal barrier film may be gold, platinum, rhodium or other metals characterized by a high work function value, high resistance to oxidation

2

and otherwise relatively inert, and a comparatively high vaporization temperature.

Additionally, the binder suspension wherein the insulating material is contained may be a volatile binder such as the nitrates of aluminum, magnesium, beryllium and like metals or a volatile organic binder such as ethyl cellulose, methyl methacrylate, or polyvinyl alcohol employing solvents such as water, alcohol, acetone, methyl acetate, toluene, or such volatile solvents as are appropriate for the binder selected. Moreover, the insulating material may be the oxides, silicates, or combinations thereof of such metals as aluminum, beryllium, titanium and other similar metals effectively used as insulating materials in electron discharge devices.

For a better understanding of the invention, together with other and further objects, reference is made to the following disclosure and appended claims in connection with the accompanying drawings in which:

FIG. 1 illustrates an insulated wire formed for use as a heater in an electron discharge device; and

FIG. 2 is a sectional view of an insulated wire having a barrier film thereon.

Referring to the drawings, FIGURE 1 is a folded heater having an insulated layer 7 such as aluminum oxide affixed to a refractory wire 3 such as tungsten. In FIGURE 2 is shown an insulated wire with a noble metal film 5 such as gold disposed intermediate the insulating layer 7 and refractory wire 3.

The insulated wire may be made into any conventional form such as the folded heater of FIGURE 2 and inserted within a cathode of an electron tube. It has been found that the activation and operation of an electron tube requires a heater temperature of more than 1000° C. Thus, when the insulated wire having a barrier layer 5 is used as a heater in an electron tube, the temperature required for the correct activation and processing thereof vaporizes the gold film 5 from the tungsten wire 3. The gold appears to disperse within the aluminum oxide coating 7 and to deposit upon the inner surface of the cathode. Accordingly, the high work function value and inert properties of the gold are utilized to reduce the potential current leakage properties of the aluminum oxide layer 7 and the field emission of the conventional nickel cathode inner surface. Hence, leakage currents between these elements, A.C. hum, and heater brittleness are substantially reduced during operation of the electron tube.

In the process of forming the insulated wire, the gold film 5 may be vapor deposited, electroplated, or otherwise affixed to the tungsten wire 3. Thereafter, the film covered wire may be subjected to spray, immersion cataphoretic, drag or other depositing processes wherein a volatile binder suspension of the types described above containing the appropriate insulating material is deposited on the wire. Subsequently, the wire is heated to volatilize the binder constituents, harden the insulating layer, and adhere the insulating layer to the gold film. The insulated wire may then be formed into a heater, inserted into the cathode of an electron tube, and heated to activate the cathode of the tube whereupon the gold film is vaporized from the core wire.

Specifically, the tungsten wire 3 has deposited thereon the noble metal or gold film 5 within a range of 0.2% to 4.0% by weight of the core material. A film of this thickness and continuity has been found sufficient to prevent oxidation of the tungsten wire but insufficient to adversely affect the operation or appearance of surrounding elements in an electron tube. This film covered wire then has deposited thereon a tacky aluminum nitrate binder of the type described in United States Patent No. 2,179,453 having an oxide of aluminum suspended therein. This layer coated wire is then heated in air between 600° C. and 800° C. in order to volatilize the binder constitu-

ents and adhere the aluminum oxide layer to the gold film. The tungsten wire 3 with adhering gold film 5 and aluminum oxide layer 7 may then be formed into a heater as shown in FIGURE 1, inserted into an indirectly heated cathode and raised to a temperature above 1000° C. whereupon the gold film is vaporized from the tungsten wire.

It has been found that the binder volatilization and insulator baking temperature of from 600° C. to 800° C. provides optimum adherence of the insulating materials recited above to the enumerated refractory core heater wires. Also, the conventional potentially electron emissive cathode materials like the earth metal carbonates generally require an activation temperature above 1000° C. in order to reduce to the oxides and metals necessary for the promotion of electron emission. Accordingly, the barrier noble metals, with vaporization temperatures ranging from 850° C. to 2300° C. will remain on the core wire until final tube processing.

Thus it can be seen that the gold film 5 prevents oxidation of the tungsten wire core 3 during the initial stages of the electron tube fabrication process when oxidation could otherwise readily occur. In the final stages of tube fabrication during evacuation and cathode activation the gold is vaporized in order to render the insulating aluminum oxide heater coating relatively inert and further to lower the field emission characteristics of the inside surface of the nickel cathode sleeve which surrounds the heater. Accordingly, heater cathode leakage, A.C. hum, and heater brittleness and failure are markedly reduced in the operating tube.

While there has been shown and described what are at present considered the preferred embodiments of the invention, it will be obvious to those skilled in the art that various changes and modifications may be made therein without departing from the scope of the invention as defined by the appended claims.

What is claimed is:

1. A process for forming an insulated wire adapted for use in indirectly heated electron tubes comprising the steps of depositing a film of a noble metal on a refractory wire, depositing a coating of volatile binder and aluminum oxide on said film, heating the coated wire above the volatilization temperature of the binder and below the vaporization temperature of the noble metal to cause adherence

of the aluminum oxide to the film, and subsequently heating the insulated wire to a temperature above the vaporization temperature of said noble metal.

5 2. A process for forming an insulated wire adapted for use in indirectly heated electron tubes comprising the steps of depositing a film of gold on a tungsten wire, depositing a coating of volatile binder and aluminum oxide on said film, heating the coated wire above the volatilization temperature of the binder and below the vaporization temperature of the gold to cause adherence of the aluminum oxide to the gold film, and subsequently heating the insulated wire to a temperature above the vaporization temperature of said gold.

10 3. A process for forming an insulated wire adapted for use in indirectly heated electron tubes comprising the steps of depositing upon a tungsten wire a gold film having a range of 0.2% to 4.0% by weight of said wire, depositing a coating of volatile binder and aluminum oxide on said film, heating the coated wire above the volatilization temperature of the binder and below the vaporization temperature of the gold to cause adherence of the aluminum oxide to the gold film, and subsequently heating the insulated wire to a temperature above the vaporization temperature of said gold.

15 4. An insulated wire adapted for use in indirectly heated electron tubes comprising a core of refractory wire, a layer of aluminum oxide and a volatile binder, and a barrier film of noble metal intermediate said wire and said layer.

20 5. An insulated wire adapted for use in indirectly heated electron tubes comprising a core of refractory wire, a layer of aluminum oxide and a volatile binder, and a barrier film of noble metal with a range of 0.2° to 4.0% by weight of the refractory wire intermediate said wire and said layer.

25 6. An insulated wire adapted for use in indirectly heated electron tubes comprising a core of tungsten wire, a layer of aluminum oxide, and a barrier film of gold with a range of 0.2% to 4.0% by weight of the tungsten wire intermediate said wire and said layer.

References Cited in the file of this patent

UNITED STATES PATENTS

835,938 Cazin ----- Nov. 13, 1906